

# United States Patent

[11] 3,537,488

[72] Inventor **Robert N. LeBoeuf**  
**Columbia, South Carolina**  
[21] Appl. No. **763,428**  
[22] Filed **Sept. 27, 1968**  
[45] Patented **Nov. 3, 1970**  
[73] Assignee **Uniroyal, Inc.**  
**New York, New York**  
**a corporation of New Jersey**

|           |        |                    |          |
|-----------|--------|--------------------|----------|
| 2,423,910 | 7/1947 | Snow et al. ....   | 139/409  |
| 2,793,151 | 5/1957 | Arnett.....        | 161/90X  |
| 2,794,450 | 6/1957 | Gatzke.....        | 139/411  |
| 2,799,916 | 7/1957 | Hindle.....        | 139/409X |
| 3,148,710 | 9/1964 | Rieger et al. .... | 139/415  |
| 3,197,021 | 7/1965 | Williams.....      | 139/411X |
| 3,296,062 | 1/1967 | Truslow.....       | 139/426X |
| 3,446,252 | 5/1969 | Maxham.....        | 139/415X |

Primary Examiner—James Kee Chi  
Attorney—David B. Miller

[54] **REINFORCING FABRIC**  
8 Claims, 13 Drawing Figs.

[52] U.S. Cl..... **139/415,**  
161/90  
[51] Int. Cl..... **D03d 11/00**  
[50] Field of Search..... **139/408-**  
**415, 426, 420, 383; 161/90, 91**

[56] **References Cited**  
UNITED STATES PATENTS  
Re. 25,406 6/1963 Byrne et al..... **139/412X**

**ABSTRACT:** A fabric particularly adapted for use as a reinforcement for belting, hose walls, and the like, although the fabric also can be used wherever a fabric is subjected to relatively large loads, as in the case of automotive seat belts, for example. The fabric includes basic warp yarns and binder warp yarns as well as weft yarns extending across the warp yarns. The basic warp yarns of the fabric of the invention have a crimp which is less than 2 percent and which preferably is no greater than 1 percent, so that these basic warp yarns are virtually without any crimp.



Patented Nov. 3, 1970

3,537,488

Sheet 1 of 2



FIG. 1



FIG. 2



FIG. 3



FIG. 4

FIG. 5



FIG. 6



FIG. 8



FIG. 7



FIG. 9



FIG. 11



FIG. 10



FIG. 12



FIG. 13

## REINFORCING FABRIC

## BACKGROUND OF THE INVENTION

The present invention relates to fabrics capable of withstanding relatively large tensile stresses.

Such fabrics are incorporated into conveyor belts, for example, for reinforcing purposes, or they may be incorporated in tubular form in hose walls to reinforce the latter. Also, they may be used for such purposes as automotive seat belts, for example.

Among the problems encountered with fabrics of this type is the excessive elongation which occurs under load. It is highly desirable to provide a lightweight fabric which will have an extremely small elongation under load, but up to the present time these results have been achieved only to a limited extent. Other problems encountered with fabrics of this type reside in such factors as the provision of a reliable bond between the fabric and the structure which it reinforces.

## SUMMARY OF THE INVENTION

It is accordingly a primary object of the present invention to provide a fabric capable of achieving an extremely low elongation under load as compared to similar conventional fabrics.

In particular, it is an object of the present invention to provide a fabric of this type which is of a relatively light weight while still having an extremely low elongation when under load.

Furthermore, it is an object of the invention to provide a fabric the properties of which can be determined by the properties of the yarns which make up the fabric rather than by the manner in which the fabric is woven.

Also, it is an object of the invention to provide a fabric the structure of which lends itself to achievement of an extremely reliable bond between the fabric and material in which it is embedded.

According to the invention, the fabric is composed of basic warp yarns and binder warp yarns as well as weft yarns which extend across the warp yarns. The basic warp yarns of the fabric of the invention have a crimp which is less than 2 percent and which preferably is no greater than 1 percent.

## BRIEF DESCRIPTION OF THE DRAWINGS

The invention is illustrated by way of example in the accompanying drawings which form part of this application and in which:

FIG. 1 is a transverse section of the fabric of FIG. 4 taken along line 1-1 of FIG. 4 in the direction of the arrows;

FIG. 2 is a longitudinal section of the fabric of FIG. 4 taken along line 2-2 of FIG. 4 in the direction of the arrows;

FIG. 3 is a longitudinal section of the fabric of FIG. 4 taken along line 3-3 of FIG. 4 in the direction of the arrows;

FIG. 4 is a schematic, fragmentary plan view of the fabric of FIGS. 1-3, showing the fabric at an enlarged scale;

FIG. 5 is a weave diagram of the fabric of FIGS. 1-4;

FIG. 6 is a harness draft for the fabric of FIG. 5, using six harnesses;

FIG. 7 is a harness draft for the fabric of FIG. 5 using four harnesses;

FIG. 8 is a chain draft for the fabric of FIG. 5 and harness draft of FIG. 7;

FIG. 9 is a weave diagram of a tubular woven fabric of the invention;

FIG. 10 is a harness draft of the fabric of FIG. 9 using eight harnesses;

FIG. 11 is a chain draft of the fabric of FIG. 9 and harness draft of FIG. 10;

FIG. 12 is a weave diagram of a hose fabric using the chain draft of FIG. 11; and

FIG. 13 is a harness draft of the fabric of FIG. 12 using eight harnesses.

## DESCRIPTION OF PREFERRED EMBODIMENTS

Referring to FIGS. 1-4, the fabric illustrated therein is composed of a group of basic warp yarns 20a and 20b as well as a second group of basic warp yarns 20c and 20d. In addition, the fabric has a group of binder warp yarns 22a and a second group of binder warp yarns 22b.

This fabric of the invention has three groups of weft yarns 24a, 24b, and 24c.

As is apparent from FIGS. 1-4, all of these yarns are woven to form a single ply of fabric with the groups of weft yarns 24a and 24b being respectively situated at the opposed exterior surfaces of the single ply. These outer groups of weft yarns 24a and 24b are arranged with the yarns of one of these groups aligned with and situated directly opposite the yarns of the other group to form successive pairs of directly opposed exterior weft yarns, as is apparent from FIGS. 2 and 3. The third group of weft yarns 24c respectively alternate with the pairs of aligned weft yarns and are situated inwardly of the exterior surfaces of the fabric.

The group of binder warp yarns 22a are interwoven only with the group of weft yarns 24c and the outer group of weft yarns 24b, while the other group of binder warp yarns 22b are interwoven only with the inner group of weft yarns 24c and the other outer group of weft yarns 24a. Moreover, as is apparent from FIG. 1, the group of binder warp yarns 22a respectively alternate with the group of binder warp yarns 22b. These alternating binder warp yarns are arranged in successive pairs with the yarns 22a and 22b of each of the successive pairs of binder warp yarns located directly next to each other.

However, the basic warp yarns 20a-20d are situated between the successive pairs of binder warp yarns. These basic warp yarns are arranged with the group 20a, 20b situated on

one side of the group of weft yarns 24c between the latter and the outer group of weft yarns 24a, while the other group of basic warp yarns 20c, 20d is situated on the other side of the inner group of weft yarns 24c between the latter and the other outer group of weft yarns 24b. Between the successive pairs of

binder warp yarns, each pair of basic warp yarns 20a and 20b are located directly next to each other on one side of the group of weft yarns 24c, while between successive pairs of the binder warp yarns a pair of basic warp yarns 20c and 20d are also located directly next to each other. These basic warp yarns are arranged with the basic warp yarns 20b and 20c on opposite sides of the weft yarns 24c situated directly opposite each other while the basic warp yarns 20a and 20d are situated respectively closer to successive pairs of binder warp yarns than the opposed basic warp yarns 20b and 20c.

It is thus apparent with the fabric of the invention there are twice as many basic warp yarns as binder warp yarns. Also, in the fabric of the invention the basic warp yarns are situated inwardly of the exterior surfaces of the fabric at a neutral axis of the single ply thereof so that in this way an extremely good flex life is achieved for the fabric of the invention.

Moreover, due to the nature of the weave there will be an extremely good adhesion with an elastomer in which the fabric of the invention is embedded because the elastomer will have free access to the interstices of the weave. The surface of this fabric can be very easily coated and it has a good hook pullout due to the nature of the interlocking type of construction. The fabric of the invention has excellent dimensional stability and has extremely good impact resistance due to the arrangement of the primary or basic warp yarns.

As may be seen from the weave diagram of FIG. 5, there is a repeat on six warps and three wefts. The No. 1 and 2 warps of FIG. 5 respectively correspond to the binder warp yarns 22b and 22a, while the No. 3-6 warps of FIG. 5 respectively correspond to the basic warp yarns 20a, 20b, 20c and 20d. The No. 1 weft of FIG. 5 corresponds to a weft yarn 24c, the No. 2 weft of FIG. 5 corresponds to a weft yarn 24b, and the No. 3 weft corresponds to weft yarn 24a.

The yarns may be straight drawn on six harnesses as indicated in FIG. 6, or they may be arranged in a pattern draw

on four harnesses as indicated in FIG. 7, providing in this way the chain draft indicated in FIG. 8.

FIG. 9 illustrates a weave diagram for a tubular woven fabric of the invention, while FIG. 10 shows a pattern draw for this fabric on eight harnesses and FIG. 11 shows the chain draft for the weave diagram of FIG. 9 and pattern draw of FIG. 10.

FIG. 12 is a weave diagram particularly suited for a hose fabric. The fabric of FIG. 12 is made with the chain draft of FIG. 11 and with a pattern draw of eight harnesses as shown in FIG. 13.

With the fabric of the invention the basic warp yarns 20a-20d have virtually no crimp. As a result there is an extremely low fabric elongation under load because these basic warp yarns are the load-supporting components. Because of this feature a lesser amount of basic warp yarn is required for a given length of fabric so that an extremely light weight fabric can be produced. The single ply of fabric lends itself to use as reinforcing for single ply rubber or plastic industrial conveyor belting applications.

Examples of fabrics constructed according to the invention have the characteristics indicated in table I, as follows:

TABLE I

|                   | Fabric A | Fabric B |
|-------------------|----------|----------|
| Percent Crimp:    |          |          |
| Warp (Basic)      | 1.0      | 1.0      |
| Warp (Binder)     | 81.0     | 80.8     |
| Weft              | 2.6      | 2.7      |
| Percent Take Up*: |          |          |
| Warp (Basic)      | 1.0      | 1.0      |
| Warp (Binder)     | 44.8     | 44.7     |
| Weft              | 2.5      | 2.6      |

\*Formula—10" mark in fabric.  

$$\frac{\text{Extended Lengths over } 10"}{10" + \text{Extended Length}} \times 100 = \text{Percent Take Up}$$

Three specimens which have the characteristics set forth in table I above were made and tested as indicated in table II, as follows:

TABLE II

[200# Rated Belt Fabric (having approximately 10 to 1 safety factor) Warp-Basic-1,260/4 filament nylon twisted mfg.  $\times 1.5$  T.P.I. Warp Binder-840/2 Filament Nylon twisted Mfg.  $\times 1.5$  T.P.I. Filling-1260/3 Filament Nylon twisted Mfg.  $\times 1.5$ . Weave-6 Harness]

Ends/Inch:  
 Basic—28  
 Binder—14  
 Picks/Inch—29.7  
 Ozs./Sq. Yd.—37.62  
 Gauge (in.)—0.0190

|                           | Percent,<br>Spec. 1 | Elongation,<br>Spec. 2 | Warp sample,<br>Spec. 3 | 1" wide*<br>average |
|---------------------------|---------------------|------------------------|-------------------------|---------------------|
| Applied Load at lbs.:     |                     |                        |                         |                     |
| 50                        | 0.5                 | 0.5                    | 1.0                     | 0.7                 |
| 100                       | 0                   | 1.0                    | 2.0                     | 1.3                 |
| 200                       | 2.5                 | 2.5                    | 3.5                     | 2.8                 |
| 400                       | 5.0                 | 5.0                    | 6.5                     | 5.5                 |
| 600                       | 6.5                 | 6.5                    | 8.5                     | 7.2                 |
| 800                       | 8.0                 | 8.0                    | 9.0                     | 8.3                 |
| 1,000                     | 9.0                 | 8.5                    | 10.0                    | 9.2                 |
| 1,500                     | 10.5                | 10.5                   | 11.5                    | 10.8                |
| 2,000                     | 12.5                | 12.0                   | 13.5                    | 12.7                |
| Elong. at break (percent) | 14.5                | 14.0                   | 15.0                    | 14.5                |
| Strength at break (lbs.)  | 2,280               | 2,350                  | 2,310                   | 2,313               |

\*40 Ends:  
 2" ravel strip ravelled to 1". Instron Tensile-11" jaw distance.  
 1"/min. chart and crosshead speed, used Indian Grip Jaws, (Fabric overlaps itself).

UNITED STATES PATENT OFFICE  
CERTIFICATE OF CORRECTION

Patent No. 3,537,488

November 3, 1970

Robert N. Le Boeuf

It is certified that error appears in the above identified patent and that said Letters Patent are hereby corrected as shown below:

Column 4, after line 45, insert -- only with said third group of weft yarns and one outer group of weft yarns and a second group of binder warp yarns interwoven only with said third group of weft yarns and the other outer group of weft yarns.

7. A fabric as recited in claim 6 and wherein the yarns of said one group of binder warps yarns alternate with the yarns of the second group of binder warp yarns with said binder warp yarns arranged in pairs located directly next to each other and said pairs of binder warp yarns spaced from each other accommodate basic warp yarns between said pairs of binder warp yarns, said basic warp yarns including one pair of basic warp yarns situated on one side of said third group of weft yarns between successive pairs of binder warp yarns and a second pair of basic warp yarns situated on the other side of said third group of weft yarns also between successive pairs of binder warp yarns, so that the number of basic warp yarns is twice the number of binder warp yarns with four basic warp yarns following each pair of binder warp yarns.

8. A fabric as recited in claim 7 and wherein each pair of basic warp yarns between successive pairs of binder warp yarns are located directly next to each other with only one of each pair of basic warp yarns on one side of the third group of weft yarns being situated opposite only one of the basic warp yarns on the other side of the third group of weft yarns.

Signed and sealed this 29th day of June 1971.

(SEAL)

Attest:

EDWARD M. FLETCHER, JR.  
Attesting Officer

WILLIAM E. SCHUYLER, JR.  
Commissioner of Patents